

1

3,220,086

## PROCESS FOR TREATING WOOL FOR ANTI-FELTING PURPOSES

George Henry Taylor, Rothley, Jack H. Rowlett, Oadby, and Derek Bradley, Loughborough, England, assignors to Foister, Clay & Ward Limited, Leicester, England, a British company

No Drawing. Filed Apr. 11, 1963, Ser. No. 319,912  
Claims priority, application Great Britain, Apr. 14, 1962,

14,509/62

19 Claims. (Cl. 28—76)

(Filed under Rule 47(a) and 35 U. S. C. 116)

The present invention relates to a method of producing all classes of wool knitwear, which expression is used in a generic sense and is intended to cover, not only 15 hosiery including say, socks (sox), half-hose, three-quarter hose, and sports hose, but also various other knitted garments and articles of wearing apparel including full-fashioned outerwear and underwear, and cut outerwear and underwear made on flat or circular machines—all knitted from wool or a preponderance of wool.

The object of the invention is to provide a method of producing wool knitwear which can be satisfactorily washed over and over again in a washing machine without either the appearance of the fabric or the serviceability of the articles being in any way adversely affected. Heretofore, the continual washing of such goods made of wool in a washing machine has not been possible without undue distortion, pilling, shrinkage and felting of the knitted fabric.

In particular, an aim is to minimise the total of the relaxation shrinkage plus the milling shrinkage to as little as under the figure of 5% in the case of footwear, and 5% area shrinkage in the case of garments, after washing 5 hours in a washing machine.

The improved method of this invention comprises knitting wool knitwear more tightly than usual with yarn consisting of or including wool and having a higher or tighter twist than normal, and treating the wool for anti-shrink purposes in a process which subjects it to a higher degree of chemical anti-felting treatment than is normally the case.

The treatment of the wool may be carried out either by treating the goods after fabrication, or by treating the yarn before knitting or the wool before spinning.

Turning to the characteristic step of knitting the wool knitwear "more tightly than usual." This means that the stitch length knitted with any particular count of yarn on any of the different gauges of machines is less than would be knitted normally. Due to the fact that it is possible to knit both a wide range of stitch lengths and counts on any gauge of machine, it is essential that some means of relating the desired resultant fabric with a stitch length and count of yarn be found; this relationship is provided for in the term "Cover factor" which is now used in the hosiery industry and is defined as:

$$\text{Cover factor} = \frac{1}{\text{Stitch length} \times \sqrt{\text{count}}}$$

The count in this formula is the resultant count; this means, for example, that if a 2-fold 32s yarn were used the resultant count would be 16s.

For the present purposes fabrics of higher cover factor than is usual are produced.

Thus, for fabrics knitted on one set of needles only, that is to say plain fabrics, made on circular, flat, straight bar and circular hose machines; and also ribbed fabrics made on machines using double-ended needles such as socks and half-hose and all purl fabrics, the normal cover factor range is of the order of 1.19—1.31. For

2

the purpose of the present invention the cover factor adopted is in excess of this viz. 1.32 upwards.

For fabrics knitted on two sets of needles, that is to say all rib and interlock structures, the normal cover factor range is of the order of 1.29—1.41, but for the purpose of this invention a cover factor upwards of 1.42 is adopted.

An example illustrating the comparison between a fabric having a normal cover factor and one knitted to give a higher cover factor is to be found in the production of half-hose made from wool with a Bradford worsted count of 2/27½, on a 12 gauge circular half-hose machine of 4" diameter and equipped with 168 needles. In this case the tight stitch length would be 0.1965", derived from a course length of 33", this giving a cover factor of 1.377; in normal knitting, on the other hand, the length of yarn per course would be 35" giving a substantially longer stitch length of 0.2083" and a cover factor of 1.31.

Another example of this increase in cover factor is given by fabrics produced on a 27 gauge full-fashioning machine. Using a 2/32s worsted yarn, a normal fabric having a cover factor of 1.19 would be obtained by knitting a stitch length of 0.21". To produce a fabric in accordance with the invention it is necessary to knit a stitch length of at least 0.1893", which gives a cover factor of 1.32; a more desirable fabric may be obtained by knitting a stitch length of 0.1780" and this gives a cover factor of 1.402.

A further example of the invention is to be found in the production of rib fabrics made from 2/32s worsted yarn on a 12 gauge circular rib machine. In this instance, a normal fabric having a cover factor of 1.38 is knitted with a stitch length of 0.1812"; whereas a suitable fabric may, in accordance with this invention, be produced having a cover factor of 1.545 by knitting a stitch length of 0.1619". The minimum conditions for this fabric would be a stitch length of 0.1761", giving a cover factor of 1.42.

As regards the "higher or tighter twist" of the yarn employed in the improved method; this is achieved by increasing the turns per inch in a singles yarn and also the turns per inch in both the singles and folding twists of a two-fold yarn above that normally used in a hosiery yarn. For example, in the case of a normal singles, 64s quality wool hosiery yarn of 1/27½ Bradford worsted count, this can have a twist of 11 turns per inch which is arrived at by the simple formula:

$$\text{Turns per inch} = \frac{\text{count}}{3} + 2$$

In the improved method the singles twist is increased to that given by the formula:

$$\text{Turns per inch} = \frac{(\text{count} + 8)}{3}$$

which in this case would be 11½ turns per inch.

The folding twist of a two-fold hosiery yarn is normally up to approximately 50% of the twist used in the singles components; thus, for a 2/27½ Bradford worsted count wool yarn with a normal twist this would be 5½ turns per inch folding, and this may be arrived at by the formula:

$$\text{Turns per inch (folding)} = \frac{\text{count} + 5}{6}$$

A most important feature of the present invention is that the folding twist of the selected two-fold yarn can ideally be the same as that used in the singles components, but the minimum conditions at which the invention will work is for the folding twist of the two-fold yarn to be 75% of the twist in the single components.

An example of this is seen in the production of fully fashioned knitwear on a 27 gauge full-fashioning machine using a two-fold yarn having 13 turns per inch in the singles components and (ideally) also 13 turns per inch in the folding; however, the minimum folding twist would be 9 1/4 turns per inch based on a 64s quality wool yarn of Bradford worsted count 2/32s.

A further example is in the production of wool half-hose on a 168 needle, 12 gauge, 4" diameter machine using a 64s quality wool yarn. If two single ends of 27 1/2 Bradford worsted count are used, the turns per inch will be 11 1/4 in each yarn; if 2/27 1/2 Bradford worsted count yarn is used the turns will be 11 1/4 turns per inch in the singles components and (ideally) 11 1/4 in the folding, although a minimum folding twist would be 8.8 turns per inch.

Finally, treating the wool in such a way as to subject to a higher degree of chemical anti-felting treatment than is normally the case means that the said wool is treated for anti-felting purposes in a chemical anti-felting process in which the concentration of the reagents used is greater than is normally applied.

For example, in anti-felting processes employing chlorine as the active reagent, which may be applied either directly to the wool, or by liberation from chlorine-containing compounds—either alone or in the presence of other compounds, the percentage of chlorine which is usually applied is in the range of 2-2 1/2%. For the purpose of this invention the amount of chlorine applied to the wool will be at least 3%.

#### Method of testing

The aforementioned ranges of twists, cover factors and percentages of chemical anti-felting treatment were determined by tests carried out in a 1952 model Hoover washing machine with the impeller speed reduced to 460 r.p.m. and having an inside size of 29 cms. x 35 cms. x 34 cms. deep. 30 litres of 0.5% soap solution (using water of zero hardness) were used at 85° C. and the total weight of the goods under test was made up to 2 lbs. The duration of each test was 3 hours.

The actual method of preparing samples and the measurement of relaxation and milling shrinkage is laid down in British Standard No. 1955:1953.

The normal cover factor range is specified in the Journal of the Textile Institute, vol. 53, p. 630.

We claim:

1. A method of producing wool knitwear comprising the steps of (a) so knitting the knitwear of a two-fold wool yarn comprising two singles components on a knitting machine of a selected gauge that the resultant count of the said yarn and the length of the stitches formed therefrom gives a cover factor

$$\text{cover factor} = \frac{1}{\text{stitch length} \times \sqrt{\text{count}}}$$

exceeding 1.32 for a fabric knitted on one set of needles only and 1.42 in respect of a fabric knitted on two sets of needles, the twist in turns per inch of each singles component of the said two-fold yarn being given by the formula

$$\frac{(\text{count}+8)}{3}$$

and the folding twist of said yarn being at least 75% of the twist in the singles components, and (b) treating the wool for anti-felting purposes in a chemical anti-felting process in which chlorine is used as the active reagent and in which the concentration of available chlorine is at least 3% of the dry weight of the wool in the fabric.

2. A method of producing wool knitwear comprising the steps of (a) so knitting the knitwear of a singles yarn comprising wool on a knitting machine of a selected gauge that the resultant count of the said yarn and the

length of the stitches formed therefrom gives a cover factor

$$\text{cover factor} = \frac{1}{\text{stitch length} \times \sqrt{\text{count}}}$$

exceeding 1.32 for a fabric knitted on one set of needles and 1.42 in respect of a fabric knitted on two sets of needles, the twist in turns per inch of the singles yarn being given by the formula

$$\frac{(\text{count}+8)}{3}$$

and (b) treating the wool for anti-felting purposes in a chemical anti-felting process in which chlorine is used as the active reagent and in which the concentration of available chlorine is at least 3% of the dry weight of the wool in the fabric.

3. A method of producing wool knitwear comprising the steps of (a) knitting the knitwear of wool yarn comprising at least one singles component having a twist in turns per inch given by the formula

$$\frac{(\text{count}+8)}{3}$$

the said yarn being so knitted on a knitting machine of a selected gauge that the resultant count of the yarn and the length of the stitches formed therefrom gives a cover factor

$$\text{cover factor} = \frac{1}{\text{stitch length} \times \sqrt{\text{count}}}$$

exceeding 1.32 for a fabric knitted on one set of needles only and 1.42 in respect of a fabric knitted on two sets of needles, and (b) treating the wool for anti-felting purposes in a chemical anti-felting process in which chlorine is used as the active reagent and in which the concentration of available chlorine is at least 3% of the dry weight of the wool in the fabric.

4. A method according to claim 3, wherein the said treatment of the wool is carried out by treating the goods, after fabrication, for anti-shrink purposes.

5. A method according to claim 3, wherein the said treatment of the wool is carried out by treating the yarn prior to knitting.

6. A method according to claim 3, wherein the said treatment of the wool takes place before it is spun into the said yarn.

7. A method of producing wool half-hose comprising the steps of (a) so knitting the half-hose of a two-fold yarn having a Bradford worsted count of 2/27 1/2 on a 12 gauge circular half-hose machine having a needle cylinder of 4" diameter and equipped with 168 needles as to produce a stitch length of 0.1965", derived from a course length of 33" and giving a cover factor

$$\text{cover factor} = \frac{1}{\text{stitch length} \times \sqrt{\text{count}}}$$

of 1.377, the twist in turns per inch of each singles component of the said two-fold yarn being given by the formula

$$\frac{(\text{count}+8)}{3}$$

and the folding twist of the yarn being at least 75% of the twist in the singles components, and (b) treating the wool for anti-felting purposes in a chemical anti-felting process in which chlorine is used as the active reagent and in which the concentration of available chlorine is at least 3% of the dry weight of the wool in the fabric.

8. A method of producing wool fabric comprising the steps of (a) so knitting the fabric of a two-fold wool yarn having worsted count of 2/32s on a 27 gauge full-

fashioning machine as to produce a stitch length of at least 0.1893" giving a cover factor

$$\text{cover factor} = \frac{1}{\text{stitch length} \times \sqrt{\text{count}}}$$

of 1.32, the twist in turns per inch of each singles component of the said two-fold yarn being given by the formula

$$\frac{(\text{count} + 8)}{3}$$

and the folding twist of the yarn being at least 75% of the twist in the singles components, and (b) treating the wool for anti-felting purposes in a chemical anti-felting process in which chlorine is used as the active reagent and in which the concentration of available chlorine is at least 3% of the dry weight of the wool in the fabric.

9. A method as claimed in claim 8, which is modified to knit a stitch length of 0.1780" and give a cover factor of 1.402.

10. A method of producing a wool rib fabric comprising the steps of (a) so knitting the fabric of a two-fold wool yarn having a worsted count of 2/32s on a 12 gauge circular rib machine as to produce a stitch length of 0.1619" giving a cover factor

$$\frac{1}{\text{stitch length} \times \sqrt{\text{count}}}$$

of 1.545, the twist in turns per inch of each singles component of the said two-fold yarn being given by the formula

$$\frac{(\text{count} + 8)}{3}$$

and the folding twist of the yarn being at least 75% of the twist in the singles components, and (b) treating the wool for anti-felting purposes in a chemical anti-felting process in which chlorine is used as the active reagent and in which the concentration of available chlorine is at least 3% of the dry weight of the wool in the fabric.

11. A method of producing a wool rib fabric comprising the steps of (a) so knitting the fabric of a two-fold wool yarn having a worsted count of 2/32s on a 12 gauge circular rib knitting machine as to produce a stitch length of 0.1761" giving a cover factor

$$\frac{1}{\text{stitch length} \times \sqrt{\text{count}}}$$

of 1.42, the twist in turns per inch of each singles component of the said two-fold yarn being given by the formula

$$\frac{(\text{count} + 8)}{3}$$

and the folding twist of the yarn being at least 75% of the twist in the singles components, and (b) treating the wool for anti-felting purposes in a chemical anti-felting process in which chlorine is used as the active reagent and in which the concentration of available chlorine is at least 3% of the dry weight of the wool in the fabric.

12. A method of producing fully-fashioned knitwear comprising the steps of (a) so knitting the fabric of a two-fold 64s quality wool yarn of Bradford worsted count 2/32s having 13 turns per inch in the singles components and a folding twist of anything from 9 1/4 to 13 turns per inch on a 27 gauge full-fashioning machine as to produce a stitch length of at least 0.1893" giving a cover factor

$$\frac{1}{\text{stitch length} \times \sqrt{\text{count}}}$$

of 1.32, and (b) treating the wool for anti-felting purposes in a chemical anti-felting process in which chlorine is used as the active reagent and in which the concentration of available chlorine is at least 3% of the dry weight of the wool in the fabric.

13. A method as claimed in claim 12, which is modified to knit a stitch length of 0.1780" and give a cover factor of 1.402.

14. A method of producing wool half-hose comprising the steps of (a) so knitting the half-hose of a two-fold 64s quality wool yarn of Bradford worsted count 2/27 1/2 having 11 1/4 turns per inch in the singles components and a folding twist of anything from 8.8 to 11 1/4 turns per inch on a 12 gauge circular half-hose machine having a needle cylinder of 4" diameter equipped with 168 needles that the aforesaid count of the yarn and the length of the stitches formed from the said yarn gives a cover factor

$$\frac{1}{\text{stitch length} \times \sqrt{\text{count}}}$$

15 exceeding 1.32, and (b) treating the wool for anti-felting purposes in a chemical anti-felting process in which chlorine is used as the active reagent and in which the concentration of available chlorine is at least 3% of the dry weight of the wool in the fabric.

16. A method of producing wool half-hose comprising the steps of (a) so knitting the half-hose of a yarn comprising two ends of 1/27 1/2 Bradford worsted count 64s quality wool having 11 1/4 turns per inch in each end on a 12 gauge circular half-hose machine having a needle cylinder of 4" diameter and equipped with 168 needles that the aforesaid count of the yarn and the length of the stitches formed from the said yarn gives a cover factor

$$\frac{1}{\text{stitch length} \times \sqrt{\text{count}}}$$

17 exceeding 1.32, and (b) treating the wool for anti-felting purposes in a chemical anti-felting process in which chlorine is used as the active reagent and in which the concentration of available chlorine is at least 3% of the dry weight of the wool in the fabric.

18. A method of producing wool knitwear comprising the steps of (a) so knitting the knitwear of a two-fold wool yarn comprising two singles components on a knitting machine of a selected gauge that the resultant count of the said yarn and the length of the stitches formed therefrom gives a cover factor

$$\frac{1}{\text{stitch length} \times \sqrt{\text{count}}}$$

19 exceeding 1.32 for a fabric knitted on one set of needles only and 1.42 in respect of a fabric knitted on two sets of needles, the twist in turns per inch of each singles component of the said two-fold yarn being given by the formula

$$\frac{(\text{count} + 8)}{3}$$

20 and the folding twist of said yarn being at least 75% of the twist in the singles components, and (b) treating the wool for anti-felting purposes in a chemical anti-felting process in which chlorine is used as the active reagent and is applied directly to the wool, the percentage of such chlorine present in the process being at least 3%.

21 17. A method as claimed in claim 16, which is modified by application of the chlorine to the wool by liberation from chlorine-containing compounds.

22 18. A method of producing wool knitwear comprising the steps of (a) so knitting the knitwear of a singles yarn comprising wool on a knitting machine of a selected gauge that the resultant count of the said yarn and the length of the stitches formed therefrom gives a cover factor

$$\frac{1}{\text{stitch length} \times \sqrt{\text{count}}}$$

23 exceeding 1.32 for a fabric knitted on one set of needles only and 1.42 in respect of a fabric knitted on two sets of

needles, the twist in turns per inch of the singles yarn being given by the formula

$$\frac{(\text{count}+8)}{3}$$

and (b) treating the wool for anti-felting purposes in a chemical anti-felting process in which chlorine is used as the active reagent and is applied directly to the wool, the percentage of such chlorine present in the process being at least 3%.

19. A method as claimed in claim 18, which is modified by application of the chlorine to the wool by liberation from chlorine-containing compounds.

## References Cited by the Examiner

## UNITED STATES PATENTS

|           |        |         |       |         |
|-----------|--------|---------|-------|---------|
| 1,522,555 | 1/1925 | Trotman | ----- | 8—128   |
| 3,100,674 | 8/1963 | Steiger | ----- | 8—127.6 |

## OTHER REFERENCES

Moncrieff, "Wool Shrinkage and Its Prevention," The London Trade Press Ltd, copyrighted 1953, pages 488 and 489.

DONALD W. PARKER, Primary Examiner.